

## UNITED STATES PATENT OFFICE

2,088,674

## CLEANSING OF TEXTILE PRODUCTS

William Whitehead, Cumberland, Md., assignor  
to Celanese Corporation of America, a corpora-  
tion of DelawareNo Drawing. Application February 15, 1934.  
Serial No. 711,448

9 Claims. (CL 87—5)

This invention relates to the cleansing of textile yarns and fabrics and especially of those fabrics made from yarns containing organic derivatives of cellulose.

5 An object of the invention is the economic and expeditious production of clean textile fabrics. Other objects of the invention will appear from the following detailed description.

By employing this invention textile fabrics 10 may be readily cleansed of dirty knots, oil stains, dirt marks and loom stains. In the processing of woven, knitted or otherwise formed fabrics there are developed spots of foreign matter upon the fabrics. These spots may be caused by employees knotting the yarns with dirty hands, oil dropping from bearings of the processing machinery and from unclean bobbins, shuttles and other devices. These stains are usually oily stains of an oil or grease containing dirt, iron 15 rust, metallic salts and other foreign material. Prior to this invention it has been necessary to give fabric long and severe scouring treatments, sometimes requiring heated baths, to remove these stains. By the present method of treatment, the stains are readily removed thus saving time and it also reduces risk of injuring the fabric.

This invention also is of advantage in removing quickly and non-injirously, gums and con- 30 densation products formed by the ageing of cer-  
tain types of lubricants and coating material. The yarn is thoroughly cleansed without devel-  
oping a harsh hand or scroop.

According to this invention I treat yarns and 35 fabrics, especially those containing organic de-  
rivatives of cellulose, with a detergent that is de-  
formed in situ thus gaining an increased pene-  
tration power and forming easier emulsification  
of the dirt, oil or other contaminating matter.

40 This invention is applicable to the treatment  
of yarns and fabric of all types of material such  
as cotton, reconstituted cellulose (viscose or  
cuprammonium), silk, wool, flax, etc. It is how-  
ever especially applicable to the treatment of 45  
yarns, filaments and fabrics containing organic  
derivatives of cellulose such as the organic esters  
and ethers of cellulose. Examples of organic  
esters of cellulose are cellulose acetate, cellulose  
formate, cellulose butyrate and cellulose propionate, 50 while examples of organic cellulose ethers are  
methyl cellulose, ethyl cellulose and benzyl cel-  
lulose. The yarns may be formed of other de-  
rivatives and/or substitution products of cellulose  
55 for example the ether esters of cellulose, the

mixed esters of cellulose and such products as  
nitro-cellulose acetate.

This invention is applicable to the cleansing of filaments and yarns, under which terms are included, threads, assemblies or bundles of a number of continuous filaments which may be in parallel relationship or which may be twisted together, artificial bristles, straws, short lengths of staple fibers, or yarn spun from such staple fibers. It is of primary importance however in 10 cleansing fabrics formed from such yarns by any textile method for example weaving, warp knitting, circular knitting, knotting, netting and braiding. It is also applicable to the treatment of films, foils and sheets of cellulosic material. 15

The yarns from which the fabrics may be formed may contain besides the cellulosic base material effect materials such as pigments, filling materials, dyes or lakes, fire retardants, plasticizers, sizes and lubricants. Examples of fire 20 retardants are beta chlorophenylphthalene, triphenyl phosphate, tricresyl phosphate and the ammonium salts of boron or phosphorus. Examples of plasticizers are diethyl phthalate, dibutyl tartrate etc. Examples of lubricants are olive oil, 25 teaseed oil, mineral oil, all of which may contain preservatives and aids such as oleic acid, phenol, hexaresorcinol or cyclo hexanol etc. Other conditioning agents may be employed, for example ethoxy butyrate and other ethers and 30 esters of polyhydric alcohols. Examples of filling materials are powdered metal, powdered oxides or carbonates of metals and powdered organic materials that, when incorporated with the cellulosic material, tend to absorb light. Examples 35 of sizes are wax, gelatine, with or without hydroscopic and lubricating materials, starches, gums, resins and salts of resin acids and glycerides. These effect materials may be added to the yarns by adding same to the spinning solution from which the yarns are spun or they may be incorporated with the yarns after formation of the yarns by means of swelling agents or they may be applied to the yarns as a coating, depending on the result desired.

The fabrics may be formed of a single type of yarn or of a mixture of yarns for example a warp of silk and a weft of cellulose acetate or other combinations. The fabrics may be dyed prior to or after cleansing treatment according to this invention. Permanent sizes for the material should be applied however after cleansing, as the cleansing agents have high penetrating power and would tend to remove the sizes.

In carrying out this invention the yarn or fabric

is treated, by immersion, padding, spraying or other methods of application, with an agent that forms with caustic alkalies a detergent or soap-like emulsifying material. Agents such as oil soluble acids are preferable as these penetrate (by dissolving the oil) into the solid areas or for that matter into any layer or coating of oily material, under the dirt marks and between the dirt. These agents are then caused to react or be neutralized with alkali to form a detergent or soap-like material which will dislodge and emulsify the dirt and oil. In this manner the cleansing agent is formed in situ and uniformly throughout the contamination to be removed from the fabric. The high degree of penetration of the acid reagent causes a quick and deep emulsifying action and does not rely on progressively washing away the outer layers. By this method the cleansing agent is self accumulating where the contamination of the fabric is greatest thereby exerting little or no action on a clean part of the fabric.

The agents that form with alkalies a detergent or soap-like material that are applicable to this invention are preferably organic acids. Examples of oil soluble organic acids are oleic acid, stearic acid, palmitic acid, linoleic acid and other fatty acids and naphthenic acids such as hexahydrobenzoic acid and hexamethylene-carboxylic acid or mixtures of such acids. Other acids having similar characteristics may be employed. Naphthenic acids react very rapidly with the alkali and the soap-like material produced has very strong emulsifying powers.

Any strong base material may be employed to neutralize or partially neutralize or saponify the acid that forms a readily emulsifiable product. Examples of such base materials are sodium and potassium hydroxide, ammonia, mono-, di- and tri-amines, mono-, di- and tri-ethanolamine and other similar basic materials. It is unnecessary to add to the fabric, that has been treated with the oil soluble acid, a molecular equivalent of the neutralizing base material. A partial neutralization of the acid may be sufficient and is sometimes preferred in the treatment of fabrics containing organic derivatives of cellulose. The salt of the acid that is formed acts as an emulsifying agent to remove, besides the dirt and oil, the excess acid. For certain purposes however an excess of the alkali may be employed.

This invention is applicable to spot removing from fabrics containing organic derivatives of cellulose. Thus fabrics containing dirty knots or oil spots may be, locally, rubbed gently by hand with a naphthenic or other suitable acid and then subsequently scoured in 0.25 g. p. l. soda ash plus 1 g. p. l. soap at 75° C. The dyeing and delustering properties are not locally affected by application of the naphthenic acid to the soiled places. The concentration of the various solutions may be varied to suit each particular case. The alkaline material may be supplied to the material from an aqueous bath, an alcohol bath, a soap bath or baths containing other neutral or basic materials.

The following examples are given as description and not as limitations.

#### Example I

A fabric made of yarns of cellulose acetate, having soiled places comprising dirty oil splashes, iron contaminated oil on knots, and comparatively dry soiled knots soiled with finely divided metallic iron originating from the reed and

shuttle boxes, is padded with naphthenic acid and passed between pressure rollers to remove the excess acid leaving about 20% acid on the fabric.

The fabric is then allowed to stand 1 to 2 hours and then scoured at 75° C. in a bath containing 1 gram per liter of sodium hydroxide. To this bath additional NaOH may be added, if desired, substantially to neutralize the acid. The fabric may then be given short scourings at 75° C. in 0.25 grams per liter soda ash or weak soap solution. This final scour removes the last trace of the peculiar odor of naphthenic acid.

Other bath temperatures may be employed say from 60 to 100° C. or more, however, one of the advantages of this invention is the efficiency of cleansing in baths below 85° C. or the temperature at which organic esters of cellulose may tend to become delustered. The use of cooler baths i. e. below 85° C. has a tendency to protect the strength of the fabric if the same is later treated in a hot bath.

#### Example II

A soiled fabric, of yarns of cellulose acetate, is padded with oleic acid on a padding mangle. This fabric is treated in a scour bath at 75° C. of NaOH of a concentration sufficient to neutralize from 15 to 30% of the acid. About 20 minutes after the immersion of the fabric in the scour bath 1 cc. per liter of ammonia is added to the bath to more nearly neutralize the acid. The fabric is removed from the bath and dried. It is found to be clean and uninjured.

#### Example III

Either naphthenic acid or oleic acid is emulsified in ten times its weight of water by adding to the mixture of acid and water sufficient NH<sub>4</sub>OH to neutralize 10% of the acid and then agitating the mixture. The fabrics are padded with this emulsion, passed between pressure rollers and after standing from 1 to 2 hours is scoured in a bath containing 0.5 grams per liter soda ash. In this way 3 to 4% of acid is applied to the fabrics.

The acid may be applied to the fabric in amounts of from 2 to 30% on the weight of the fabric. The amount employed will depend upon the type and constituents of the fabric treated, the degree of contamination and the method of application. The acid may remain on the yarn or fabric from 0.5 to 12 hours or longer without detrimental effects. The treatment in the baths will be about 20% shorter when employing naphthenic acids and sodium hydroxide than when employing other acids.

Having described my invention what I desire to secure by Letters Patent is:

1. Method of washing textile materials containing cellulose esters, which comprises applying thereto an acid which forms a detergent soap with a strong base and thereafter subjecting the materials to the action of an aqueous bath containing such base in quantity sufficient to neutralize a part only of the acid on the materials.

2. Method of washing textile materials containing cellulose acetate, which comprises applying thereto an acid which forms a detergent soap with a strong base and thereafter subjecting the materials to the action of an aqueous bath containing such base in quantity sufficient to neutralize a part only of the acid on the materials.

3. Method of washing textile materials containing cellulose esters, which comprises applying

2,088,674

thereto an acid which forms a detergent soap with strong bases and thereafter subjecting the materials to the action of a dilute aqueous bath containing a base, selected from the group consisting of alkali and ammonium hydroxides and amines, in quantity sufficient to neutralize a part only of the acid on the materials.

4. Method of washing textile materials containing cellulose acetate, which comprises applying thereto an acid which forms a detergent soap with strong bases and thereafter subjecting the materials to the action of a dilute aqueous bath containing a base, selected from the group consisting of alkali and ammonium hydroxides and amines, in quantity sufficient to neutralize a part only of the acid on the materials.

5. Method of washing textile materials containing cellulose esters, which comprises locally applying to soiled parts of said materials an oil-soluble acid which is at most only slightly soluble in water and which forms a detergent soap with a strong base and thereafter subjecting the materials to the action of an aqueous bath containing such strong base in quantity sufficient to neutralize a part only of the acid on the materials.

6. Method of washing textile materials containing cellulose acetate, which comprises locally applying to soiled parts of said materials an oil-soluble acid which is at most only slightly soluble in water and which forms a detergent soap with

a strong base and thereafter subjecting the materials to the action of an aqueous bath containing such strong base in quantity sufficient to neutralize a part only of the acid on the materials.

7. Method of washing textile materials containing cellulose esters, which comprises locally applying to soiled parts of said materials a fatty acid which forms a detergent soap with a strong base and thereafter subjecting the materials to the action of an aqueous bath containing such strong base in quantity sufficient to neutralize a part only of the free acid on the materials.

8. Method of washing textile materials containing cellulose acetate, which comprises locally applying to soiled parts of said materials a fatty acid which forms a detergent soap with a strong base and thereafter subjecting the materials to the action of an aqueous bath containing such strong base in quantity sufficient to neutralize a part only of the free acid on the materials.

9. Method of washing textile materials containing cellulose acetate, which comprises locally applying to soiled parts of said materials a naphthenic acid which forms a detergent soap with a strong base and thereafter subjecting the materials to the action of an aqueous bath containing such base in quantity sufficient to neutralize a part only of the free acid on the materials.

WILLIAM WHITEHEAD. 30